# EUROPEAN PATENT SPECIFICATION

(11) **EP 0 733 316 B1**
(45) Date of publication and mention of the grant of the patent: **02.08.2000**
(21) Application number: 96302032.6
(22) Date of filing: 25.03.1996
(51) Int. Cl.: A44C 21/00

(54) **Coins and methods for producing coins**
Münze und Verfahren zu ihrer Herstellung
Pièces de monnaie et leurs procédés de fabrication

(30) Priority: 23.03.1995 GB 9505920
(43) Date of publication of application: 25.09.1996
(73) Proprietor: The Solicitor for the Affairs of Her Majesty's Treasury, Llantrisant, Mid Glamorgan, CF7 8YT (GB); THE UNIVERSITY OF LIVERPOOL, Liverpool L69 3BX (GB)
(72) Inventor: Hatherley, Peter Graham, Bridgend, Mid Glamorgan, CF35 6HD (GB); Watkins, Kenneth Gordon, Wirral, Merseyside, L48 3HF (GB); Steen, William Maxwell, Caldy, Wirral, Merseyside, L48 1NB (GB)
(74) Representative: Gibson, Stewart Harry

(56) References cited:
- DE-A- 2 644 018
- DE-A- 3 204 445
- DE-A- 3 207 405
- DE-A- 4 240 886
- DE-U- 9 400 167
- US-A- 4 322 601

## Description

The present invention relates to coins and more particularly to the formation of designs or patterns in the surfaces of coins.

In recent years, coinage across the world has been increasingly manufactured by electroplating a surface layer over a core or substrate material, usually of mild steel. Steel coins plated with nickel, copper, brass or bronze are now used in numerous countries world-wide. In a smaller number of cases, nickel or zinc has been chosen as the core material. In addition, certain coins have been manufactured from coated ("clad") strip, with steel, nickel, cupro-nickel or copper being used as in the inner layer.

Hitherto, there has been a limitation in the issue of coins of high value since features that could be added for authentication at a cost commensurate with the value of the coin have been capable of forgery.

It is one object of the present invention to provide a process for providing coins with authentication features that cannot easily be reproduced.

It is another object of the present invention to provide a process for providing coins with machine-readable features that can be used for authentication in coin-operated machinery or in machine-operated coin authentication systems.

DE-3207405 discloses a coin comprising a substrate of a first material and one or more coating layers, and carrying a design or pattern. This known design or pattern is formed by laser welding small plate-like particles of nickel onto the outer circumferential surface of the coin, and then pressing the particles into said surface.

According to a first aspect of the present invention, there is provided a process for producing a design or pattern in the surface of coins, comprising the steps of pre-coating a substrate of a first material with a single coating layer or a plurality of coating layers, said coating layer or layers being of a material or materials which differ from the material of said substrate, and applying a high power laser beam to define the required design or pattern over the coated surface of said substrate such as to produce localised melting of the material of said coating layer and the material of said substrate, or of the materials of said coating layers, the localised melting of the materials in the required design or pattern under the action of said laser beam being such that mixing of the materials takes place substantially only in these localised regions so as to produce a measurable or observable difference in optical, electrical or magnetic properties between transformed and untransformed regions.

The transformation achieved as a result of the localised melting can involve full or partial alloying of metal materials or other changes in the structures of the materials which result in said measurable or observable differences in optical, electrical or magnetic properties between the transformed and untransformed regions.

Preferably where there are two or more different coating layers applied to the substrate, no melting of the substrate material is involved.

The pre-coating step can be carried out by any suitable process, including electro deposition, physical vapour deposition, chemical vapour deposition, roll bonding, or other suitable conventional coating techniques or combination of techniques.

The substrate can be a metal, such as steel, or an alloy, or, in the case of multiple coating layers, any other suitable carrier material.

The coating layers are preferably different elemental metals or metal alloys but could also be other materials such as ceramic or glasses or superconducting or semiconducting materials.

The laser beam can be moved relative to the substrate material or vice versa, whichever is more convenient, to achieve the required pattern or design. Alternatively, or in addition, the pattern or design can be achieved by the use of one or more masks placed over the target material or disposed directly in the optical system of the laser.

In a preferred embodiment, the observable difference between the transformed and untransformed regions takes the form of a visible distinction in colour between these regions.

The process in accordance with this invention can produce differences of other physical properties between the patterned material and the surrounding material such as optical, electrical or magnetic properties which act as a barrier to forgery and which permit automatic recognition in vending machines or bank counting and sorting machines, particularly as a means of establishing the authenticity of the coin. For example, this could include the production of optical features such as a difference in the specularity of patterned regions on the surface of the coin which could be used by the public as a readily visible mark of the authenticity of the coin.

Another example consists in the formation of a bar code as a means of recognition. This can be achieved, for example, by selection of the types of materials in the predeposited layers in order that the required difference in properties with untransformed material is displayed in the transformed regions produced by the laser.

The parameters of the laser alloying process are preferably determined for the suitable control of the composition of the resulting alloy layers by pre-selecting the depth of melting and the relative thickness of the coating layer or layers.

For example, with any laser capable of causing surface melting of the coated starting materials (for example, but not exclusively, CO₂, CO, Nd:YAG, Nd:glass lasers;GaAs,AlAs,AlGaAs and other solid state diode lasers; liquid dye or ruby lasers, Ti:sapphire lasers - these lasers operating in continuous or pulsed mode or Q:switched mode) and with combinations of predeposited layers of thickness of 0.1-1000 µm and with laser power in the range 10-10,000 W or pulsed energy in the range 0.1-1000 Joules/pulse and laser spot size of 0.1-20 mm and substrate rate of movement beneath the laser beam of 0.1-1000 mm/s, alloyed layers of depth 0.1-1000 µm can be created at specific regions on the surface. In this way the chemical composition of the alloyed layer can be controlled by selection of the laser process parameters and the relative thickness of the pre-coated layers. Control of the above parameters also allows control of the melt depth and the melt width and hence the physical dimensions of the laser alloy pattern produced.

The process of the invention produces patterns in the alloy layers by a control of the degree of absorption of the laser energy during processing as a result of the application of a laser energy absorbent coating on the surface which is applied only to those areas where absorption is required (and hence for alloying to take place). Hence, for example, a dark coloured or other coloured absorbent coating may be applied by any conventional printing process in the pattern or design which is required. Because of the high selectivity of absorption of laser energy between treated and untreated regions, when the laser is scanned across the surface of the material which has been coated with successive layers of constituent alloy material as described above, the pattern is reproduced as a laser alloy printed design in the surface (as a result of alloying taking place only in those regions beneath the absorbent coating layer).

According to a second aspect of the invention, there is provided a coin comprising a substrate of a first material, the substrate having a single coating layer or a plurality of coating layers, said coating layer or layers being of a material or materials which differ from the material of said substrate, and carrying a design or pattern, the coin being characterised in that said design or pattern is formed by localised melting of the material of said coating layer and the material of said substrate, or of the materials of said coating layers.

The invention is described further hereinafter, by way of example only, with reference to the accompanying drawings, in which:
Fig. 1 illustrates a typical laser arrangement by which the present technique can be performed;
Fig. 2a is a sectional view illustrating a substrate carrying two surface coatings of different metals prior to laser treatment;
Fig. 2b is a sectional view, corresponding to Fig. 2a, showing the condition following laser treatment; and
Fig. 3 (a) to (f) show examples of some possible designs that can be produced in coins using the technique of the present invention.

The apparatus of Fig. 1 includes a laser 10, a mask 12, an angled mirror 14 and an X-Y support table 16 for carrying a sample object 18 to be patterned. The laser beam is indicated at 19 and is arranged to deliver sufficient energy to melt the coating layer(s) on the substrate and promote alloying (or mixing) only in the areas where the design is required. When the resulting alloy is a different colour to the outer layer on the substrate, a visible printed design is thereby produced.

This apparatus is in itself conventional and has been used already for laser ablation and laser engraving techniques. Indeed, several processes are known at the present time for the production of alloys on the surface of metallic and other material, using the action of a laser on a pre-coated layer of another material on a substrate which is mixed with the substrate on melting to form an alloy, these processes being known generically as laser surface alloying. However, none of these processes has the object of creating alloying in restricted regions of the surface in order to produce a design or pattern resulting from the difference in colour, optical, magnetic, electrical, superconducting or semiconducting properties of the design compared with the unalloyed surrounding material, for the production of patterning or recognition features in coins.

It should be noted that the process performed by the apparatus of Fig. 1 can equally well be operated without a mask 12, producing a pattern by moving the X-Y table beneath the laser beam 19.

In the example shown in Fig. 2, a steel substrate 20 is first provided with thin coatings of nickel 22 and copper 24 by any of the techniques described hereinbefore and within the thickness ranges specified. After laser operation, a localised stripe 26 is formed which consists of a Cu-Ni alloy: this has a different colour to the surrounding copper and is therefore clearly visible to the naked eye as a means of identification for example, for authentication purposes.

The process of Fig. 2 can equally well work with a single metal layer on the substrate, in which case the material of the single metal layer is alloyed with material from the adjacent portion of the substrate to produce the required alloying. It will be noted that this is distinguished from known laser engraving techniques since the latter do not seek to achieve melting and alloying, but instead achieve total removal of the engraved material. By use of the present invention, localised melting and alloying of the superposed materials creates a different type of structure in a finely restricted zone enabling the latter zone to be exploited as an ornamentation or as a security device, or as both, as described hereinbefore.

Ornamental effects rely on the visible contrast in the colours of metals and alloys. Historically, there have been three basic colours used for metallic coinage - red, yellow and white. If it is required to maintain use of those colours, the present technique could be used to provide alloys from an appropriate combination of materials from the following categories:

| RED | YELLOW | WHITE |
|---|---|---|
| For example: | For example: | For example: |
| Copper | Gold | Silver |
| | Brass (Cu-Zn) | Cupro-Nickel |
| | Bronze (Cu-Sn) | Nickel |
| | Aluminium Bronze (Cu-A1) | Nickel Silver |
| | | Silver, |

The coloured trace generated by the laser might be a simple line or geometric pattern. Alternatively, as an ornamental feature, it could be used to highlight certain features in the coin design such as the effigy, the date or the edge beading.

From the point of view of security, the presence of a localised visible trace generated in the surface of the coin by the present invention serves to enhance the intrinsic security of the coin. It will be difficult for a counterfeiter to attempt to reproduce the feature without recourse to a similar very expensive laser device. Furthermore, it would be no easy matter to impart the trace in a finished coin. In the application of the present process, the laser processing is carried out before the coin has been struck, i.e. on a flat blank.

The presence of a detectable trace in the surface can serve to authenticate a coin in much the same way as a watermark or metal thread is used in a banknote. However, the surface trace in the coin can also be designed to be detected by an automatic coin validator in vending machines, bank counting and sorting machines and the like.

A machine-readable feature need not require that the trace be of contrasting colour. For example if cupro-nickel (the silver-coloured alloy presently used for such denominations such as the British 50p or the German 1 DM) is plated with a layer of nickel, the laser can be used to generate a localised cupro-nickel alloy at the surface. This trace will not contrast in colour but, when the coin is carefully examined, the trace is just visible by virtue of its slightly different hue. More importantly, however, the physical properties of the coin are disrupted locally so that it becomes possible to detect this in a suitably adapted coin validator.

Most coin validators today are electronic devices in which the coin passes a series of coils operating at various frequencies. The presence of the coin alters the resonant frequency of these coils and the amplitude of the signal.

The shift in one, or other, or both of these parameters serves to characterise the coin being tested. The highest frequency coils are used to detect the surface properties of the coin, and the lower frequencies for the interior. These devices are thus particularly well suited to the new generation of plated coins, because in principle both of the metallic components can be distinguished in this way.

Figure 3 show diagrammatically examples of possible designs that can be produced in coins using the method of the present invention. Figure 3(a) shows a single stripe 30. Figure 3(b) shows a double stripe 31,32. Figure 3(c) shows a barcode 33 (which may be either a magnetic or optical barcode). Figure 3(d) shows a pattern 34 in the form of the date (in this case the calendar year of production of the coin). Figure 3(e) shows a design 35 in the form of a head. Figure 3(f) shows a pattern 36.

## Claims

1. A coin comprising a substrate (20) of a first material, the substrate (20) having a single coating layer (22) or a plurality of coating layers (22,24), said coating layer (22) or layers (22,24) being of a material or materials which differ from the material of said substrate (20), and carrying a design or pattern, the coin being characterised in that said design or pattern is formed by localised melting of the material of said coating layer (22) and the material of said substrate (20), or of the materials of said coating layers (22,24).

2. A coin as claimed in claim 1, characterised in that the material of said substrate (20) and the materials of said coating layer (22) or layers (22,24) are metallic, whereby said design or pattern is formed by one or more alloyed regions of the melted materials.

3. A coin as claimed in claim 1 or claim 2, characterised in that said design or pattern formed by the localised melted region or regions comprises a stripe (30) or stripes (30,32).

4. A coin as claimed in claim 3, characterised in that said stripes (30,32) form a magnetic or optical barcode.

5. A coin as claimed in claim 1 or claim 2, characterised in that said design or pattern formed by the localised melted region or regions comprises a geometric pattern and/or an ornamental pattern (35).

6. A process for producing a design or pattern in the surface of coins, comprising the steps of pre-coating a substrate (20) of a first material with a single coating layer (22) or a plurality of coating layers (22,24), said coating layer (22) or layers (24) being of a material or materials which differ from the material of said substrate (20), and applying a high power laser beam (19) to define the required design or pattern over the coated surface of said substrate (20) such as to produce localised melting of the material of said coating layer (22) and the material of said substrate (20), or of the materials of said coating layers (22,24), the localised melting of the materials in the required design or pattern under the action of said laser beam (19) being such that mixing of the materials takes place substantially only in these localised regions so as to produce a measurable or observable difference in optical, electrical or magnetic properties between transformed and untransformed regions.

7. A process as claimed in claim 6, wherein said substrate (20) is pre-coated with a plurality of coating layers (22,24) and the required design or pattern is produced by localised melting of said coating layers (22,24), characterised in that no melting of the material of said substrate (20) takes place.

8. A process as claimed in claim 6 or claim 7, characterised in that the material of said coating layer (22) or layers (22,24) is or are metallic.

9. A process as claimed in claim 8, characterised in that the pre-coating step is carried out by electro deposition, physical vapour deposition, chemical vapour deposition, or roll bonding, or a combination of any of the latter techniques.

10. A process as claimed in any of claims 6 to 9, characterised in that the material of said substrate (20) is metallic.

11. A process as claimed in any of claims 6 to 9, characterised in that the material of said substrate (20) is non-metallic.

12. A process as claimed in claim 11, characterised in that said substrate (20) is made of a ceramic, glass, superconducting or semi-conducting material.

13. A process as claimed in any of claims 6 to 12, characterised in that the required pattern is defined over the coated surface of said substrate (20) by moving said laser beam (19) relative to the material of said substrate (20).

14. A process as claimed in any of claims 6 to 12, characterised in that the required pattern is defined over the coated surface of said substrate (20) by moving the material of said substrate (20) relative to said laser beam (19).

15. A process as claimed in any of claims 6 to 12, characterised in that the required pattern is defined over the coated surface of said substrate (20) by positioning a mask in the path of said laser beam (19).

16. A process as claimed in any of claims 6 to 12, characterised in that the required pattern is defined over the coated surface of said substrate (20) by applying an additional laser energy absorbent coating only on those areas where absorption is required.

17. A process as claimed in any of claims 6 to 16, characterised in that the material of said substrate (20) and/or of the coating layer (22) or layers (22,24) is selected so that said observable difference between the transformed and untransformed regions takes the form of a visible distinction in colour between these regions.

18. A process as claimed in any of claims 6 to 17, characterised in that said design or pattern is arranged to be in the form of a barcode.

19. A process as claimed in claim 10 appended to claim 8, characterised in that the parameters of the alloying process achieved by the mixing of the materials are determined for the suitable control of the composition of the resulting alloy layers by pre-selecting the depth of melting and the relative thickness of said coating layer or layers.

## Patentansprüche

1. Münze, die ein Substrat (20) aus einem ersten Material aufweist, wobei das Substrat (20) eine einzige Beschichtung (22) oder eine Mehrzahl von Beschichtungen (22,24) aufweist, wobei die Beschichtung (22) oder Beschichtungen (22,24) aus einem Material oder Materialien besteht bzw. bestehen, das bzw. die sich vom Material des Substrats (20) unterscheidet bzw. unterscheiden und eine Gestaltung oder ein Muster tragen, wobei die Münze dadurch gekennzeichnet ist, daß die Gestaltung oder das Muster durch lokalisiertes Schmelzen des Materials der Beschichtung (22) und des Materials des Substrats (22) oder der Materialien der Beschichtungen (22,24) gebildet ist.

2. Münze nach Anspruch 1, dadurch gekennzeichnet, daß das Material des Substrats (20) und das Material der Beschichtung (22) oder Beschichtungen (22,24) metallisch ist bzw. sind, wodurch die Gestaltung oder das Muster durch einen legierten Bereich oder mehrere legierte Bereiche der geschmolzenen Materialien gebildet ist.

3. Münze nach Anspruch 1 oder 2, dadurch gekennzeichnet, daß die Gestaltung oder das Muster, das durch den lokalisierten geschmolzenen Bereich oder die Bereiche gebildet ist, einen Streifen (30) oder Streifen (30,32) aufweist.

4. Münze nach Anspruch 3, dadurch gekennzeichnet, daß die Streifen (30,32) einen magnetischen oder optischen Strichcode bilden.

5. Münze nach Anspruch 1 oder 2, dadurch gekennzeichnet, daß die Gestaltung oder das Muster, das durch den lokalisierten geschmolzenen Bereich oder die Bereiche gebildet ist, ein geometrisches Muster und/oder ein Schmuckmuster (35) aufweist.

6. Verfahren zum Herstellen einer Gestaltung oder eines Musters in der Oberfläche von Münzen, das die Schritte aufweist, ein Substrat (20) eines ersten Materials mit einer einzigen Beschichtung (22) oder einer Mehrzahl von Beschichtungen (22,24) vorher zu beschichten, wobei die Beschichtung (22) oder Beschichtungen (24) aus einem Material oder Materialien ist bzw. sind, das bzw. die sich vom Material des Substrats (20) unterscheidet bzw. unterscheiden, und einen Laserstrahl (19) hoher Leistung anzuwenden, um die erforderliche Gestaltung oder das erforderliche Muster über die beschichtete Oberfläche des Substrats (20) zu bestimmen, um so lokalisiertes Schmelzen des Materials der Beschichtung (22) und des Materials des Substrats (20) oder der Materialien der Beschichtungen (22,24) zu bewirken, wobei das lokalisierte Schmelzen des Materials in der erforderlichen Gestaltung oder dem erforderlichen Muster unter Wirkung des Laserstrahls (19) so ist, daß Mischen der Materialien im wesentlichen nur in diesen lokalisierten Bereichen stattfindet, um so einen meßbaren oder beobachtbaren Unterschied in optischen, elektrischen oder magnetischen Eigenschaften zwischen umgewandelten und nicht umgewandelten Bereichen zu erzeugen.

7. Verfahren nach Anspruch 6, bei dem das Substrat (20) vorher mit einer Mehrzahl von Beschichtungen (22,24) beschichtet ist und die erforderliche Gestaltung oder das erforderliche Muster durch lokalisiertes Schmelzen der Beschichtungen (22,24) bewirkt wird, dadurch gekennzeichnet, daß kein Schmelzen des Materials des Substrats (20) stattfindet.

8. Verfahren nach Anspruch 6 oder 7, dadurch gekennzeichnet, daß das Material der Beschichtung (22) oder Beschichtungen (22,24) metallisch ist.

9. Verfahren nach Anspruch 8, dadurch gekennzeichnet, daß der Schritt des Vorher-Beschichtens durch elektrolytische Fällung, physikalische Dampfablagerung, chemische Dampfablagerung oder Rollbonden oder eine Kombination einer dieser Techniken durchgeführt wird.

10. Verfahren nach einem der Ansprüche 6 bis 9, dadurch gekennzeichnet, daß das Material des Substrats (20) metallisch ist.

11. Verfahren nach einem der Ansprüche 6 bis 9, dadurch gekennzeichnet, daß das Material des Substrats (20) nichtmetallisch ist.

12. Verfahren nach Anspruch 11, dadurch gekennzeichnet, daß das Substrat (20) aus einem keramischen, Glas-, supraleitenden oder halbleitenden Material hergestellt ist.

13. Verfahren nach einem der Ansprüche 6 bis 12, dadurch gekennzeichnet, daß das erforderliche Muster über die beschichtete Oberfläche des Substrats (20) durch Bewegen des Laserstrahls (19) relativ zum Material und dem Substrat (20) bestimmt wird.

14. Verfahren nach einem der Ansprüche 6 bis 12, dadurch gekennzeichnet, daß das erforderliche Muster über die beschichtete Oberfläche des Substrats (20) dadurch bestimmt wird, daß das Material des Substrats (20) relativ zum Laserstrahl (19) bewegt wird.

15. Verfahren nach einem der Ansprüche 6 bis 12, dadurch gekennzeichnet, daß das erforderliche Muster über die beschichtete Oberfläche des Substrats (20) dadurch bestimmt wird, daß eine Maske in den Weg des Laserstrahls (19) gebracht wird.

16. Verfahren nach einem der Ansprüche 6 bis 12, dadurch gekennzeichnet, daß das erforderliche Muster über die beschichtete Oberfläche des Substrats (20) dadurch bestimmt wird, daß eine zusätzliche Laserenergie absorbierende Beschichtung nur auf den Bereichen aufgebracht wird, wo Absorption erforderlich ist.

17. Verfahren nach einem der Ansprüche 6 bis 16, dadurch gekennzeichnet, daß das Material des Substrats (20) und/oder der Beschichtung (22) oder Beschichtungen (22,24) so ausgewählt wird, daß der beobachtbare Unterschied zwischen den umgewandelten und nicht umgewandelten Bereichen die Form einer sichtbaren Unterscheidung in der Farbe zwischen diesen Bereichen hat.

18. Verfahren nach einem der Ansprüche 6 bis 17, dadurch gekennzeichnet, daß die Gestaltung oder das Muster so ausgebildet ist, daß es die Form eines Strichcodes hat.

19. Verfahren nach Anspruch 10 in Abhängigkeit von Anspruch 8, dadurch gekennzeichnet, daß die Parameter für das Legierungsverfahren, das durch das Mischen der Materialien erreicht wird, für geeignete Steuerung der Zusammensetzung der resultierenden Legierungsschichten bestimmt werden, indem die Tiefe des Schmelzens und die relative Dikke der Beschichtung oder Beschichtungen vorher ausgewählt werden.

## Revendications

1. Une pièce de monnaie comprenant un substrat (20) en un premier matériau, le substrat (20) ayant une couche (22) de revêtement unique ou une pluralité (22, 24) de couches de revêtement, cette couche (22) ou ces couches (22, 24) de revêtement étant en un matériau ou des matériaux qui différent du matériau dudit substrat (20) et portant un dessin ou modèle,
la pièce de monnaie étant caractérisée en ce que ledit dessin ou modèle est formé par fusion locale du matériau de ladite couche (22) de revêtement et du matériau dudit substrat (20), ou bien des matériaux desdites couches (22, 24) de revêtement.

2. Une pièce de monnaie telle que revendiquée à la revendication 1,
caractérisée en ce que le matériau dudit substrat (20) et les matériaux de ladite couche (22) ou desdites couches (22, 24) de revêtement sont métalliques, grâce à quoi ledit dessin ou modèle est formé par une ou plusieurs régions alliées des matériaux fondus.

3. Une pièce de monnaie telle que revendiquée à la revendication 1 ou la revendication 2,
caractérisée en ce que ledit dessin ou modèle formé par la ou les régions fondues localement comprend une raie (30) ou des raies (30, 32).

4. Une pièce de monnaie telle que revendiquée à la revendication 3,
caractérisée en ce que lesdites raies (30, 32) forment un code-barres magnétique ou optique.

5. Une pièce de monnaie telle que revendiquée à la revendication 1 ou la revendication 2,
caractérisée en ce que ledit dessin ou modèle formé par la ou les régions fondues localement comprend un modèle géométrique et/ou un modèle ornemental (35).

6. Un procédé de production d'un dessin ou modèle dans la surface de pièces de monnaie, comprenant les étapes de pré-revêtement d'un substrat (20) en un premier matériau par une couche (22) de revêtement unique ou une pluralité de couches (22, 24) de revêtement, ladite couche (22) ou lesdites couches (24) de revêtement étant en un matériau ou des matériaux qui différent du matériau dudit substrat (20), et application d'un faisceau laser multi-kilowatt (19) pour définir le dessin ou modèle requis sur la surface revêtue dudit substrat (20) apte à produire une fusion localisée du matériau de ladite couche (22) de revêtement et du matériau dudit substrat (20), ou bien des matériaux desdites couches (22, 24) de revêtement, la fusion localisée des matériaux dans le dessin ou modèle requis sous l'action dudit faisceau laser (19) étant telle qu'un mélange des matériaux a lieu sensiblement seulement dans ces régions localisées de manière à produire une différence mesurable ou observable des propriétés optiques, électriques ou magnétiques entre les régions transformées et non transformées.

7. Un procédé tel que revendiqué à la revendication 6, dans lequel ledit substrat (20) est pré-revêtu d'une pluralité de couches (22, 24) de revêtement et le dessin ou modèle requis est produit par fusion localisée desdites couches (22, 24) de revêtement,
caractérisé en ce qu'aucune fusion du matériau dudit substrat (20) n'a lieu.

8. Un procédé tel que revendiqué à la revendication 6 ou la revendication 7,
caractérisée en ce que le matériau de ladite couche (22) ou desdites couches (22, 24) de revêtement est ou sont métalliques.

9. Un procédé tel que revendiqué à la revendication 8,
caractérisé en ce que l'étape de pré-revêtement est effectuée par déposition électrolytique, déposition physique en phase vapeur, déposition chimique en phase vapeur ou fixation par laminage, ou par une combinaison de quelconques de ces dernières techniques.

10. Un procédé tel que revendiqué à l'une quelconque des revendications 6 à 9,
caractérisé en ce que le matériau dudit substrat (20) est métallique.

11. Un procédé tel que revendiqué à l'une quelconque des revendications 6 à 9,
caractérisé en ce que le matériau dudit substrat (20) est non métallique.

12. Un procédé tel que revendiqué à la revendication 11,
caractérisé en ce que ledit substrat (20) est constitué d'une céramique, d'un verre, d'un matériau supraconducteur ou semi-conducteur.

13. Un procédé tel que revendiqué à l'une quelconque des revendications 6 à 12,
caractérisé en ce que le modèle requis est défini sur la surface revêtue dudit substrat (20) en déplaçant ledit faisceau laser (19) par rapport au matériau dudit substrat (20).

14. Un procédé tel que revendiqué à l'une quelconque des revendications 6 à 12,
caractérisé en ce que le modèle requis est défini sur la surface revêtue dudit substrat (20) en déplaçant le matériau dudit substrat (20) par rapport audit faisceau laser (19).

15. Un procédé tel que revendiqué à l'une quelconque des revendications 6 à 12,
caractérisé en ce que le modèle requis est défini sur la surface revêtue dudit substrat (20) en positionnant un masque sur le trajet dudit faisceau laser (19).

16. Un procédé tel que revendiqué à l'une quelconque des revendications 6 à 12,
caractérisé en ce que le modèle requis est défini sur la surface revêtue dudit substrat (20) en appliquant un revêtement additionnel absorbant l'énergie laser seulement sur les aires où une absorption est requise.

17. Un procédé tel que revendiqué à l'une quelconque des revendications 6 à 16,
caractérisé en ce que le matériau dudit substrat (20) et/ou de la couche (22) ou des couches (22, 24) de revêtement est sélectionné de telle manière que ladite différence observable entre les régions transformées et non transformées prend la forme d'une distinction de couleur visible entre ces régions.

18. Un procédé tel que revendiqué à l'une quelconque des revendications 6 à 17,
caractérisé en ce que ledit dessin ou modèle est agencé pour être sous la forme d'un code-barres.

19. Un procédé tel que revendiqué à la revendication 10 jointe à la revendication 8,
caractérisé en ce que les paramètres du processus d'alliage accompli par le mélange des matériaux sont déterminés pour le contrôle convenable de la composition des couches d'alliage résultantes en pré-sélectionnant la profondeur de fusion et l'épaisseur relative de ladite couche ou desdites couches de revêtement.
